

## UNITED STATES PATENT OFFICE.

GEORGE L. BIDWELL, OF RIEGELSVILLE, PENNSYLVANIA, ASSIGNOR TO THE WARREN MANUFACTURING COMPANY, OF RIEGELSVILLE, NEW JERSEY, A CORPORATION OF NEW JERSEY.

## PROCESS OF MAKING PULP FOR PAPER.

No Drawing.

Application filed March 1, 1920. Serial No.362,325.

*To all whom it may concern:*

Be it known that I, GEORGE L. BIDWELL, a citizen of the United States of America, and a resident of Riegelsville, in the county of 5 Bucks and State of Pennsylvania, have invented a new and useful Process of Making Pulp for Paper, of which the following is a specification.

My invention relates to improvements in 10 processes of producing pulp from "hard stock" for use in the manufacture of paper, and consists generally and broadly in dusting, cooking, and washing the hard stock in large pieces, in reducing such pieces, in 15 bleaching and washing the reduced hard stock, and in keeping the latter in a state of hydration until the same is ready for the paper-making machine or said machine is ready for the pulp, all as hereinafter set 20 forth.

The two more important features of my 25 process reside in the utilization of comparatively large pieces of hard stock, or, in other words, in treating the stock in large pieces during a considerable period of the pulp-making process, and in maintaining the stock in a state of hydration until used, for 30 reasons which presently will be made plain, and the steps in the process incident to producing or resident in said features are both new and novel.

One object of my invention is to produce 35 a hard-stock pulp, for use in the manufacture of paper, that can be handled in slush form, as in the manufacture of paper from soft stock, due to the fact that said pulp is maintained in an advanced stage or high state of hydration, to the end that a large and important saving is effected in time, 40 raw material, power, labor, floor space, lime, bleach, etc. With this process complete control of the hydration of the fibres of the stock is both possible and practical, and any of the hard-stock elements can be rapidly 45 converted into pulp which is suitable for either the coarse grades or the finest grades of coating, drawing, writing, map, ledger, bank-note, and similar papers, and ready at any time for the beater through which the 50 pulp passes before it reaches the paper-making machine.

Another object is so to treat hard stock with water and maintain the same in a state

of hydration that the resultant pulp is thoroughly protected or preserved by a viscosity produced by the water in combination with the fibrous elements, and kept ready for instant use at all times. I control the hydration of the stock or fibre from the time the stock is cooked, or first washed, provided 55 washing precedes the cooking, as may be the case, until said stock is run into the paper-making machine. And I do not subject the stock to pressure, or have to employ manual labor in the actual handling of the 60 stock after the same is fed into the cooking and washing machine, which latter consists of an open-top engine preferably of the Hollander type.

Still another object is to produce a hard- 65 stock pulp from which can be made a cleaner paper than is possible with pulp produced by the old process or any modification of the same, and give to the finished paper superior characteristics that cannot be obtained under the old process. The afore- 70 said superior characteristics are due to the viscous bodies produced in the pulp by the long continued action of the water on the hard stock, to the action of said water on 75 said stock throughout a number of steps in the process, and to the fact that hydration of the fibre is not permitted to become lost or even lessened.

A further object is greatly to simplify the 80 hard-stock process and correspondingly to enhance or increase the efficiency and practicability of the same.

Other objects and advantages will appear 85 in the course of the following description.

It is to be understood that some latitude is permissible in the number and order or sequence of the steps of the process, so long as the scope of what is claimed be not exceeded.

In order better to understand the new process and be able to distinguish clearly the differences between the old and the new processes, it is deemed expedient to describe as briefly as may be the old process, and this I will proceed to do before taking up the new process in detail. The old process has been in use for 75 years or more without modification of the fundamental principle, although attempts have been made to modify said process in minor and unimportant 100 105

details, and patents have been issued for variations in said process. Fundamentally, however, the old process remains the same, as just observed.

5

*Old process.*

The old process of making paper or paper pulp from hard stock preliminarily consists in sorting, cutting, dusting, cooking, washing, bleaching and draining. A mellow "half stuff" is thus produced which is allowed to season in the drainer, and is then dug out, loaded into small hand-cars, carried to the beater engine, and furnished to 10 the latter by hand. The steps of sorting consists in handling the hard stock to remove therefrom buckles, buttons, and all other foreign materials and substances. After the stock is sorted it is fed into a 15 rag cutter and reduced to small pieces. The action of the rag cutter produces much lint which represents a loss of fibre when the stock is subjected to the dusting step. The cut and reduced stock is led by an apron 20 conveyor into what is termed a "railroad" duster, and thence into a cylinder duster. The purpose of the dusting operations produced by said dusters is to remove all the 25 dust from the stock, and such purpose is most effectually attained, but unfortunately 30 the two machines take out with the dust and dirt a considerable quantity of lint, as just intimated, which represents a direct loss 35 of stock, as much as 8% of the original weight of the hard stock being lost at this point.

From the cylinder duster the hard stock 40 is led by another apron conveyor to a closed cooker in the form of a rotary boiler. This 45 boiler is of either of the well-known cylindrical or spherical type, and mounted to rotate very slowly, or about three revolutions per minute. About three tons of stock may be placed in such boiler or cooker. As the 50 charge of stock is aproned into the cooker, a cooking solution of caustic soda, milk or lime, or a mixture of lime and carbonate of soda is added. The cooker is then sealed, steam is admitted, the steam pressure being 55 of from ten to forty pounds, and said cooker is rotated for from three to fourteen hours, the cooking solution, the pressure of the steam, and the time of the cook all depending on the grade of paper that is to be made from the hard stock.

The large pieces of hard stock that I use 60 in the new process could not be successfully cooked in the rotary boiler or cooker and in the manner just explained, because such pieces would roll up and would not cook.

After cooking the hard stock for the required length of time, the steam is shut off, and the cooker is blown to reduce the pressure so that said cooker can be opened. The 65 steam escapes through the customary "blow-

off", and a considerable amount of good fibre passes off with the steam and cooking liquor through said blow-off and is wasted, in spite of the presence of a strainer over the blow-off.

70

When the cooker is opened, by the removal of its "man-heads", said cooker is caused to revolve and the hard stock is automatically dumped on the floor under the cooker, a certain amount escaping therefrom 75 at each revolution. The cooker will not entirely empty itself in this manner, consequently the services of an attendant are required to "pull" the balance of the contents of the cooker, which is work of a very hot, 80 disagreeable, and arduous nature.

The hard stock is now permitted to cool and season, either under the cooker, or in a bin to which the entire "cook" is removed, the handling of the stock incident to the removal thereof hastening the cooling of the same. The too sudden cooling of the stock, however, makes it very difficult to wash and hard to bleach. After seasoning, the 85 stock is taken to a washing engine in small 90 hand-cars, and thoroughly washed to remove all the dirt and residue of the liquor. The washed stock is bleached to the desired degree of whiteness with chloride of lime or bleaching powder, after which all traces 95 of the bleaching solution are removed by washing the stock in a drum washer. And the stock is finally discharged into cement or porous tile drainers which permit the water to drain off. The stock is now known 100 as "half-stuff" and is ready for the beating operation.

From the time the bale of hard stock is broken open until the half-stuff is dug from the drainer from four to ten days must 105 elapse.

The old process involves a great amount of labor, inasmuch as the stock has to be handled and rehandled at every stage or step of the way, and handled and rehandled at a 110 disadvantage. Such process is also very uneconomical because of the waste due to the fact that the fundamental principle of cleaning is wrong, and to the continuous or frequent handling. Furthermore chemicals 115 used in the cooking and bleaching steps of the process are wasted because of the crude manner in which they are applied. And most important of all is the loss sustained because of the partial hydration of the fibre, 120 under the old process, and the loss of power, for be it remembered half-stuff is drained and held in drainers to mellow and season so that more or additional time and power are necessary in the heater in order to re-establish the desired and necessary degree of hydration. The hydration of the fibre is an absolute essential in order to form up a sheet of paper on the paper-making machine, consequently any degree of hydration once ob- 125 130

tained should be retained until the pulp is formed into paper. This fact is self-evident. Lastly it may be mentioned that time, labor, and power are wasted by the use of the rag cutters, dusters, rotaries or cookers, and drainers which are essential to the old process.

I employ in the new process cooking solutions similar to those employed in the old process and which are well known except that such a solution in the present case is in a very dilute state because of the presence in the Hollander engine in which said solution is placed of a larger volume of water than can be contained or worked in a rotary cooker in the old process, and because, furthermore, of the thorough agitation which takes place in said engine. The initially finely cut stock in the rotary cooker takes up more room than the coarser stock in the Hollander engine, proportionately, and the circulation in the former is altogether too slow to be effective.

The steam in my process is introduced into the Hollander engine and preferably to an extent only which brings the contents of said engine to a degree of temperature that is just below the boiling point.

The Hollander engine is utilized very largely in the new process. Not only is the steam introduced into the Hollander engine, and previously thereto the cooking solution, but the cooking solution is washed away from said engine, the hard stock is reduced to a pulp therein, and the bleaching and final washing are done therein and therewith. The cooking solution or liquor extracts entirely the sizing, lignin, etc. from the fibre.

The new process will now be described in detail.

#### *New process.*

The hard stock is first sorted and the pieces which are approximately a yard square or less are thrown on to an apron conveyor, while the pieces which exceed that dimension are placed in a rag chopper before being delivered to said conveyor. In the chopper the large pieces are cut, by means of a slowly revolving axe knife which shears against a bed knife, into pieces about a yard square, and the pieces so cut are dropped from said chopper on to the aforesaid conveyor. In the old process the stock is practically shredded, by means of knives or blades constructed and arranged to that end, into small pieces, with the result that a large amount of lint is produced and the edges of said pieces are frayed, which entails a material loss that is obviated by the chopping operation, and by leaving the stock in comparatively large pieces. The stock in the first instance, if of the proper size, and in the second instance, after being

chopped to the proper size, is received from the above-mentioned conveyor on an apron conveyor in the bottom of an enclosed whipper-house.

In the whipper-house the stock is thoroughly dry cleaned. The stock being in large pieces, the amount of waste during the dry-cleaning operation or step in the process is also a negligible quantity. After being dry cleaned the stock is carried to a Hollander engine especially adapted for use in the present process.

The equipment of the Hollander engine is of such a nature that the hard stock can therein be cooked and washed, or washed, cooked, and rewashed, cut into or reduced to fine particles, bleached, and again washed, all of which coupled with the novel features of the new process enables one to produce, after only eight hours treatment, a most excellent pulp of a length that can be readily pumped.

From the Hollander engine the pulp is emptied into stuff-chests where it is agitated and held in reserve until supplied to the beaters. This storing of the pulp in a high state of hydration in the stuff-chests may be said to constitute the final step in the new process as a whole.

The Hollander engine used in carrying out my process, and by means of which said engine becomes a very valuable and important auxiliary element in said process, has a specially constructed beater roll, a washing cylinder covered with #30 (in place of #60) wire mesh, sand grades which are coarser, and sand traps which have an extra large area and are extra deep. More dirt can be removed through #30 than through #60 wire mesh, which is the reason for using the former. The sand grates are 50% coarser in this case, and the sand traps are twice as large in area, and twice as deep, in the Hollander engine which I use than they are in the ordinary Hollander engine, in order to facilitate the dropping of the dirt into the sand traps and enable them to receive and contain all of said dirt, there being dirt here that in the old process would be removed by the rag dusters. The beater roll must have no wood or material in its construction that will not withstand the action of heat and of the chemicals used in the process. This roll revolves in contact with the usual bed plate or bed-plate knife, and is kept in motion from the time the hard stock is first immersed in the water in the Hollander engine until said stock as pulp ready for the beater is removed from said engine, and during all this time the stock is subjected to the reducing action of said roll, and is at atmospheric pressure in the water.

The first step in the process, so far as the Hollander engine is concerned, may be that

of washing, or it may be that of cooking, depending upon the amount of dirt in the hard stock, and to some extent on the nature or character of said stock. Although this preliminary washing is not as a rule necessary, for the purpose of this description it will be assumed that the stock is first washed, which is done by turning on the wash water to the Hollander engine, and continuing the washing operation for upwards of an hour or so long as is required to clean the stock. The wash water is next shut off and the water in the engine allowed to wash down so that the stock circulates freely and properly, the washing down being effected with the aid of the washing cylinder of the engine which is lowered and caused to dip out the dirty water and discharge it to and through the waste. Fresh water is admitted to the engine during the time the dirty water is being discharged.

The beater roll is revolving meanwhile and continues to revolve until the stock becomes pulp and is removed from the Hollander engine, said roll operating constantly to cause the stock to circulate and also reduce said stock to an ever increasing degree of fineness, so to speak.

After the first washing the stock is subjected to the action of the steam and the cooking solution, the former being then turned on to the engine and the latter being introduced into said engine. The cooking solution here is in a very much more diluted state, on account of the presence of a much larger volume of water, than could be worked in the rotary cooker of the old process, and of the thorough agitation to which said water is subjected by the beater roll, as hereinbefore pointed out. The following is a comparison of two ordinary formulas for cooking solutions:

For the cook in the Hollander engine (new process)—

45      16,212    lbs. of water,  
       1,200    "    stock,  
       132    "    lime,  
       1½    "    caustic soda.

50      For the cook in the rotary cooker (old process)—

55      19,437    lbs. of water,  
       6,000    "    stock,  
       800    "    lime,  
       1.8    "    caustic soda.

From this will be obtained an idea of the ratio of dilution of the solutions.

The above-mentioned chemicals are well known to those skilled in the art of cooking hard stock. In my process I merely cut down the quantity, as already stated. The application of these chemicals in the Hollander engine, where they can be thoroughly agitated and circulated with the

hard stock while the latter is being steamed apart, not only completely cooks the fibre, frees the lignin, and leaves said fibre mellow and pliable, but has a decided bleaching effect or action as well, which is a matter 70 possessing considerable advantage and importance.

Steam is introduced through the side of the Hollander engine preferably at a point about six inches above the floor of the engine and opposite to the end of the mid-feather. And the steam is blown into the engine for about one and one-half hours, when it is shut off. The stock is now permitted to circulate, always under the impetus or impulsion which the mass in the engine receives from the revolving beater roll, for about one-half hour in the hot cooking liquor, at the end of which time it is found that the stock is thoroughly cooked and the lignin separated from the fibre, all without bringing the contents of the engine to the boiling point.

The rewashing or second washing, where there has been a previous washing as in the present example, follows the cooking, and this is accomplished with the aid of the washing cylinder. Except when in use the washing cylinder is in elevated and inactive position, but when in use said cylinder is lowered to dip out the dirty water, as previously explained, fresh water being admitted to the engine at the same time the dirty water is being discharged. This washing is continued until the cooking liquor is all washed away and a very bright, well cooked pulp is obtained, which is ready to be bleached. Some three hours are usually required for the removal of the cooking solution.

The term "pulp" applied in the preceding paragraph to the stock is used advisedly because said stock has by this time been reduced to a pulpy condition by the action of the beater roll operating against the bed 110 knife of the engine, by the disintegrating action of the cooking liquor, and by the circulation, it having then been "worked out of the rag" and into a fibrous state.

The continual admissions of fresh water to the engine, during the washing operation after the cooking operation, washes away through the washing cylinder the cooking liquor, and with it the lignin, natural coloring matter, and sizing agents, leaving a 115 bright pulp which can readily be bleached with chloride of lime, a less quantity of said lime being required than with the old method of cooking in the old process.

Next to the final operation or step of the process in the Hollander engine is that of bleaching. This is accomplished with the usual bleaching liquor which is introduced into the circulating mass of pulp in the engine, after the cooking liquor has been 120 125 130

washed away. The action of the bleaching liquor is similar in this case to that in a case under the old process, except that a less quantity is needed, and a better intermix-  
5 ture of the pulp and liquor is made possi-  
ble, for reasons already plainly set forth. The bleaching operation takes but a com-  
paratively short time.

The final operation or step in the Hollander engine is that of washing the bleaching liquor from the pulp, or, in other words, in rewashing said pulp. This is done in a manner similar to that previously described in full, the washing cylinder being employed  
10 as upon the other occasions. All of the above-described steps which take place in the Hollander engine occur while the stock is in water at atmospheric pressure, as previously observed.  
15 As a final step in the process the pulp prepared in the manner hereinbefore set forth in detail is pumped or otherwise introduced into a stuff-chest or -chests and left until needed in the actual process of making paper.

The new process affords complete control of the hydration of the fibres, inasmuch as they are held in suspension in water from start to finish of the process after the Hollander engine is reached. In cooking under pressure in the old process, and draining under the rotary cooker and again in drainers, the water leaves the fibres, and when they are again placed in solution the hydration is not nearly so easily controlled. Under the new process the fibres contain a surplus of water all through the washing before cooking, if that step be included, the cooking, the washing after cooking, the bleaching, and the washing after bleaching, or right up to the time the stock or pulp is emptied into the stuff-chest, and even until said pulp is pumped into the beater to be thickened for the final treatment in the  
20 beater and refiner.

The hard stock, surcharged with water and protected by a viscosity produced by a combination of water and fibre elements, to restate an important and vital fact connect-  
25 ed with the new process, and thus reduced to a pulp in a "mushy" state, is stored as just explained in the stuff-chests until needed, when said pulp is pumped into the beater engine, the washing cylinder of such engine being utilized to make the "furnish" as dry, comparatively and technically speaking, as may be desired. From the beater engine the pulp goes to the cylinder or Fourdrinier paper-making machine. A pulp in an ad-  
30 vanced stage of hydration is produced by my process, not only without confining the stock under pressure, but without directly-applied manual labor after the stock is fed to the Hollander engine.

65 By providing several Hollander engines

which are especially equipped for use in my process, and stuff-chests and pumps located in the basement under said engines, each of the latter can be loaded with a separate kind of hard stock and given proper chemical treatment, after which any desired blend may be made in the beater engine. Thus, for example, in a mill provided with six Hollander engines, two could be run on jute, and four on rope, making a furnish in the  
70 beater which would consist of one-third jute and two-thirds rope.

My hard-stock pulp remains in a slush state like soft-stock pulp handled in a wood mill.  
80

Caustic soda and carbonate of lime have been applied to stock in a Hollander engine for the removal of ink from old papers, but not for cooking hard stock, and so far as is known lime has never been used in a  
85 Hollander engine for any purpose.

It will have been noted that the cooking, (omitting a previous washing which experience has shown to be seldom needed), washing, bleaching, and rewashing steps  
90 take place in the Hollander engine in the sequence named, while what may be termed the combined step of reducing by a cutting action the hard stock and agitating and circulating the contents of said engine is continuous throughout the period covered by  
95 said sequence, wherefor it may be said that the four comparatively short, sequential steps performed in said engine are embraced by, or interposed or interspersed in a long,  
100 fifth step. In this peculiar combination of steps reside most valuable and important features. It is by them that the hard stock is cooked and bleached, with the necessary subsequent washing away of the dirt, waste,  
105 and solution in each case, and reduced to the required degree of fineness, and at the same time hydrated and maintained in a state of hydration, so that no subsequent hydration, as would be needed in the event  
110 the stock were allowed to become dry before being stored in the stuff-chests, is demanded.

Never before my invention have large pieces of hard stock been placed in a Hollander engine and therein, in water at  
115 atmospheric pressure, cooked, bleached, washed, and reduced to pulp, and this all in one continuous process. Never before has hard stock been handled in large pieces even from the start, but on the contrary  
120 it has been reduced to small pieces as soon as it was sorted. In this and other particulars the present invention is widely different from the prior art, as well as being economical and highly efficient.  
125

Obviously, when the hard stock consists of rope, the same cannot be cut into pieces which may approximate a yard square, but it can be and is cut into corresponding lengths and these lengths or long pieces are  
130

put through the process just as is the hard stock when in pieces of large area, relatively speaking.

The term "hard stock" is used herein and in the appended claims in its technical sense, as usually understood by paper manufacturers, to define a paper stock from rags and like materials, such as burlap, gunny, rope, jute, hemp, and sisal, and as distinguished from what is technically known as "soft stock" consisting of sulphite, sulphate, ground wood, and old papers.

What I claim as my invention, and desire to secure by Letters Patent, is—

1. The process of converting hard stock into half stock, in the manufacture of paper, which comprises introducing the stock, together with the required chemicals and a considerable body of water, into a suitable reducing engine and therein cooking it at atmospheric pressure in the water while subjecting it to the action of a beater roll.

2. The process of converting hard stock into half stock, in the manufacture of paper, which comprises dry cleaning the stock and introducing it, in its varying commercial sizes up to about one yard without cutting, into a suitable reducing engine and therein cooking it at atmospheric pressure in a considerable body of water while subjecting it to the action of a beater roll.

3. The process of converting hard stock into half stock, in the manufacture of paper, which comprises cooking, washing, bleaching, and rewashing the stock at atmospheric pressure while subjecting it to the action of a beater roll and in the presence throughout of a quantity of water sufficient to hydrate and to maintain the hydration of the fibers.

4. The process of converting hard stock into half stock, in the manufacture of paper, which comprises taking the stock in commercial sizes, cut only when in sizes upwards of about a yard in length, and boil-

ing, washing, bleaching, and rewashing it at atmospheric pressure while subjecting it to the action of a beater roll and in the presence throughout of a quantity of water sufficient to hydrate and to prevent dehydration of the fibers.

5. The process of converting hard stock into half stock, in the manufacture of paper, which comprises introducing the stock into an engine of the Hollander type, open to the atmosphere, and therein cooking, washing, bleaching, and rewashing it while subjected to the disintegrating action of the engine and in the presence of a quantity of water sufficient to hydrate its fibers.

6. The process of converting hard stock into half stock, in the manufacture of paper, which comprises introducing the stock, in all commercial sizes up to about one yard without cutting, into an engine of the Hollander type, and therein cooking, washing, bleaching, and rewashing it at atmospheric pressure, while subjecting it to the beater action of the engine, and in the presence of a quantity of water sufficient to hydrate its fibers.

7. The process of converting hard stock into half stock, in the manufacture of paper, which comprises introducing the stock into an engine of the Hollander type and, while it is being beaten up therein and before its removal therefrom, cooking, washing, bleaching, and rewashing it at atmospheric pressure and in the presence of a quantity of water sufficient to hydrate its fibers, and thereafter maintaining the converted stock suspended in water sufficient to prevent dehydration of the fibers until ready for beating.

GEORGE L. BIDWELL.

Witnesses:

HENRY N. GRIFFIN,  
WARREN M. BROTHMAN.